

## UNITED STATES PATENT OFFICE

2,680,734

## PAPER TREATING RESIN

William C. Dearing, Troy, N. Y., assignor, by  
mesne assignments, to Allied Chemical & Dye  
Corporation, New York, N. Y., a corporation of  
New York

No Drawing. Application January 26, 1950,  
Serial No. 140,745

2 Claims. (Cl. 260—70)

1

This invention relates to a thermosetting composition of improved stability and water solubility that is capable of imparting greater wet strength to paper than the synthetic resins heretofore used for the impregnation of paper.

When used for imparting wet strength to paper, a synthetic resin is usually incorporated at the wet end of the paper making process, for example, in the beater or at the head box. A synthetic resin that is incorporated at the wet end of the paper making process must be capable of dilution without precipitation of the resin, and must have an affinity for the paper fibers so that a reasonably large proportion of the resin deposits on the paper fibers and so that an unreasonably large proportion of the resin is not lost in the waste water.

The principal object of the invention is to provide a thermosetting composition of improved stability and water solubility comprising a synthetic resin that has the special properties necessary to permit it to be incorporated at the wet end of the paper making process and also imparts substantially higher wet strength per unit of cost than the resins heretofore used for the impregnation of paper. More specific objects and advantages are apparent from the description, which illustrates and discloses but is not intended to limit the scope of the invention.

A product of the reaction of formaldehyde, urea and a hydroxy-substituted carboxylic acid having not more than four carbon atoms per carboxy group imparts greater wet strength to paper than the synthetic resins heretofore used, but such a reaction product, when made from ordinary commercial formaldehyde, has very low stability so that the water solubility of the reaction product rapidly decreases during storage or shipment. Thus, although the reaction product when freshly prepared is capable of imparting superior wet strength to paper, its stability is so low that it is not usable after it has been shipped from the manufacturer to the user and, therefore, it is not marketable in accordance with ordinary commercial practice.

The present invention is based upon the discovery that a composition comprising a polyhydric alcohol having not more than two carbon atoms per hydroxy group, and a product of the reaction of formaldehyde, urea and a hydroxy-substituted aliphatic carboxylic acid whose molecule has not more than eight carbon atoms and has not more than four carbon atoms per carboxy group not only imparts superior wet strength to paper but also is stable and has a

solubility in water that does not decrease materially during ordinary storage or shipment and also is higher than the water solubility would be if the glycol were omitted.

5 In the preparation of a thermosetting composition embodying the invention the formaldehyde used may be wholly or partially in the form of one of its polymers such as paraformaldehyde, but preferably is in the form of an aqueous solution (as hereinbefore described). The hydroxy-substituted carboxylic acid may be any substance whose molecule consists of a substituted straight or branched hydrocarbon chain having at least one carboxy group and at least 10 one hydroxy group, each attached to a primary, secondary, or tertiary carbon atom, and having no substituents other than carboxy and hydroxy groups, said molecule having not more than four carbon atoms per carboxy group, i. e., 15 having from one to three additional carbon atoms per carboxy group and having not more than a total of eight carbon atoms. It is preferred that the substituents be attached to primary or secondary carbon atoms. Such substances include glycolic acid, lactic acid, hydroxyglutaric acid, hydroxybutyric acid, malic acid, and tartaric acid. For the sake of brevity the term "hydroxy-substituted carboxylic acid" is used hereinafter to designate such substances. 20 The polyhydric alcohol (for the sake of brevity, hereinafter referred to as a "glycol") may be any polyhydric alkane or linear ether thereof, which is otherwise unsubstituted, and in which there are not more than two carbon atoms per hydroxy group. Such substances include glycerine, ethylene glycol, diethylene glycol,  $\alpha$ -propylene glycol, trimethylene glycol, erythritol, 25 pentaerythritol, dipentaerythritol, adonitol, arabinitol, xylitol, mannitol, sorbitol, dulcitol, and iditol. The term "glycol" is used hereinafter to designate such substances or mixtures thereof.

It is preferred that a thermosetting composition embodying the invention comprise a glycol, and a product of the reaction of formaldehyde, urea and a hydroxy-substituted carboxylic acid 30 in which carboxy radicals are neutralized with an alkali metal base (for reasons hereinafter discussed). The term "alkali metal base" is used herein to mean any alkali metal compound that gives an alkaline solution, the preferred alkali metals being sodium and potassium. Such alkali metal bases include sodium hydroxide, potassium hydroxide, sodium alcohohates such as sodium methoxide, sodium ethoxide, and sodium 35 beta-methoxyethoxide (obtained simply by dis-

solving metallic sodium in methanol, ethanol or beta-methoxy ethanol, respectively), potassium carbonate, sodium tetraborate, potassium tetraborate, and sodium bicarbonate. The preferred alkali metal bases are sodium hydroxide and potassium hydroxide. Sodium hydroxide is more desirable from the standpoint of economy.

It is preferred that the hydroxy-substituted carboxylic acid be glycolic acid. It is preferred also that the glycol contain only one carbon atom per hydroxy group (e. g., as in glycerine, ethylene glycol, erythritol) and most desirable that it be glycerine. It is desirable that the thermosetting composition of the invention be in the form of an aqueous solution, as hereinafter described.

The glycol is believed to react to some extent with the other components of the resin. Although the glycol may be mixed with the resin after it is prepared, and its mere presence in the water solution will make the resin more soluble and more stable than a resin comprising a similar reaction product whose aqueous solution contains no glycol, even better results are obtained when the glycol is reacted with the resin. It is preferable, therefore, to add the glycol during the resin preparation because reaction is then assured. A most desirable composition of the invention is a thermosetting composition comprising, in aqueous solution, a product of the reaction of glycerine, formaldehyde, urea, and glycolic acid, in which the glycolic acid is neutralized with sodium hydroxide.

In the practice of the invention not more than about 2.2 mols of formaldehyde should be used per mol of urea, and it is preferable to use not more than about 2.15 mols per mol of urea. Not less than about 1.8 mols of formaldehyde should be used per mol of urea and it is preferable to use not less than about 1.9 mols per mol of urea. It is most desirable to use about 2.12 mols of formaldehyde per mol of urea.

Not less than .05 mol of the hydroxy-substituted carboxylic acid should be used per mol of urea. It is preferable that the amount of hydroxy-substituted carboxylic acid used be not less than about .15 mol per mol of urea. It is preferable to use not more than about .25 mol of the hydroxy-substituted carboxylic acid per mol of urea. It is most desirable to use about .2 mol of the hydroxy-substituted carboxylic acid per mol of urea. Increasing the amount of the hydroxy-substituted carboxylic acid to as much as .5 mol per mol of urea tends to decrease the degree of wet strength imparted by thermosetting compositions embodying the invention.

The amount of glycol used in the practice of the present invention is preferably not greater than about 25 per cent and not less than about 10 per cent of the weight of urea employed, although amounts as large as 30 per cent or as small as 5 per cent may be used. It is most desirable to use about 20 per cent of the glycol based on the weight of urea. (The term "per cent" as used herein to refer to quantities of material means per cent by weight unless otherwise qualified.)

As hereinbefore stated, a thermosetting composition embodying the invention is capable of imparting superior wet strength to paper. Wet-strengthened paper is extremely useful in all paper products which may come in contact with water or moisture during use, for example toweling, food product wrappers, bag and wrapping paper, and map and blue print paper.

A synthetic resin for imparting wet strength to paper is desirably incorporated at the wet

end of the paper making process before the paper is made. This is known as "wet end addition," the term referring not only to addition in the beater but also to addition in the machine chest, head box, fan pump or any other desired point at the wet end of the paper making process. This more convenient and less expensive method of applying the resin to the paper results in a more porous paper which is not coated with a sealing. Since in the production of wet strength paper, the mixture at the point of resin addition ordinarily comprises a very dilute suspension of pulp in water (less than two per cent) and a synthetic resin used for imparting wet strength is usually present in this suspension in a concentration of about one to two per cent of the pulp concentration, the resin must be capable of dilution without precipitation. Such a resin should be a thermosetting composition so that it can be added in its soluble stage to disperse and dissolve throughout the paper pulp suspension at the wet end of the paper making process before the paper is made, and then can be converted to a thermoset resin on the paper fibers by heating during drying or ageing during storage.

Although theoretically ordinary urea-formaldehyde resins are soluble in the concentration range required during wet end addition, in actual practice these thermosetting resins form curds when incorporated at the wet end under the slightly acid conditions used, before they have had time to be dispersed and dissolved in water. The curds cannot be readily dissolved and stick to the apparatus so that much of the resin is deposited on the apparatus or lost in the waste water. (The formation of curds necessitates frequent cleaning of the apparatus and leads to serious difficulties, because under the acid conditions used the curds, after depositing on the equipment are converted to the insoluble state.) The small amount of resin that does cling to the paper fibers does not coat them uniformly. Such a resin makes the paper non-absorbent and is undesirable for use in imparting wet strength to paper.

Since urea-formaldehyde resins when used as paper treating resins to impart a high degree of wet strength must be sufficiently water soluble to dissolve so rapidly that curds do not form it is necessary to use a modifying agent which gives a high degree of water solubility to such resins. It has been found that this is accomplished by the presence of an ionic charge attached to the resin molecule, which gives it an electrical charge when in solution. The hydroxy-substituted carboxylic acid, or a salt thereof, used in the practice of the present invention becomes part of the resin through its hydroxy substituent. The ionization in solution of the substituted carboxylic acid which is thus a part of the resin molecule imparts a negative electric charge to the molecule. Such a soluble anionic resin imparts wet strength to paper when it is converted to a thermoset resin on the paper fibers by heating during drying or ageing during storage. It is believed that the presence of the solubilizing groups in the resin molecules on the fiber also imparts greater absorbency to the paper since the soluble resin is less water repellent and hence facilitates passage of water through the thin layer of resin on the fiber. The known sodium bisulfite modified resins do not have as good water solubility and do not impart as high a degree of wet strength to paper per pound of resin used as a synthetic

resin formed by the reaction of formaldehyde, urea, and a hydroxy-substituted carboxylic acid having not more than four carbon atoms per carboxy group. A thermosetting resin embodying the present invention, comprising a glycol in addition to the product of the reaction of formaldehyde, urea and a hydroxy-substituted carboxylic acid having not more than four carbon atoms per carboxy group, not only imparts a high degree of wet strength to paper, but also possesses greater stability and water solubility than the synthetic resins heretofore used for imparting wet strength to paper (as is herein-after demonstrated).

Sodium bisulfite may be used along with the hydroxy-substituted carboxylic acid in the practice of the invention. Such a modifying agent should not be present in a concentration greater than about 30 per cent of the hydroxy-substituted carboxylic acid, since its use in larger concentrations tends to give a compound of the invention which imparts lower wet strength to paper than the compounds formed by using only the hydroxy-substituted carboxylic acid.

The quantity of a thermosetting resin embodying the invention used to treat paper pulp is within the range ordinarily used in the art of making wet-strengthened paper and varies with the degree of wet strength desired. For example, the minimum desirable concentration of resin is the smallest concentration that gives an appreciable increase in the wet strength of the paper (i. e., about 0.1 per cent resin based on the weight of dry pulp). The maximum desirable concentration of resin (i. e., about 10 per cent based on the weight of dry pulp) is that above which the wet strength imparted to paper is not increased enough to make a larger concentration of resin economical for most applications. A concentration between about 0.25 and about 5 per cent ordinarily gives considerable wet strength economically and efficiently. The paper pulp used may be of any type such as bleached or unbleached sulphite, kraft or ground wood pulp. The resin may be added to the pulp at the wet end of the paper machine as prepared (i. e., as an approximately 50 per cent water solution) or, if desired, it can be diluted to about 20 per cent solids, preferably with water at a temperature above 50 degrees F. The liquid resin is infinitely dilutable with water and will, therefore, be easily and uniformly dispersed throughout the stock in the beater, machine chest, fan pump, head box or any other desired point at the wet end of the paper machine, preferably after all fiber refinement. It is desirable to add a catalyst such as alum or aluminum chloride about five minutes before the resin addition. The resin and catalyst may stand on the pulp for a few hours before the mixture is used for making paper. Such contact time should not, however, approach as long a period as 24 hours since a portion of the wet strength is lost under such conditions. The pH of the mixture should be adjusted within a range of 4.0 to 5.5, the pH being lowered to this range using for example, dilute sulfuric acid. It is most desirable that the pH of the mixture be about 4.5.

The wet strength imparted by a thermosetting resin of the invention is affected when the pH of the pulp suspension prior to the addition of the resin is varied. The hardness in the water used to dilute the pulp suspension is another factor which affects wet strength.

In the production of a thermosetting composi-

tion embodying the invention the reaction medium consists of water, usually that present in a commercial formaldehyde solution, which ordinarily is an aqueous solution consisting of 37 per cent formaldehyde and 63 per cent water. The only other source of water in the reaction mixture is that present, if any, in the hydroxy-substituted carboxylic acid, which may contain about 30 per cent of water. Further dilution during the reaction is undesirable, since it results in resins having decreased stability.

Resins embodying the invention reacted at the concentration of solids achieved using an ordinary commercial formaldehyde solution and the molar proportions of reactants hereinbefore described have greater stability and water solubility than resins heretofore known for imparting wet strength made from ordinary commercial formaldehyde. The degree of water solubility of resins used for imparting wet strength is dependent upon the number of solubilizing groups which become part of the resin molecule. Since using an amount of hydroxy-substituted carboxylic acid above the desirable limit hereinbefore described tends to decrease the wet-strengthening properties of compositions embodying the invention, it is not desirable to increase the amount of hydroxy-substituted carboxylic acid above such limit to improve the water solubility of the resins. It has been discovered that less dilution during the reaction, i. e., reacting at a higher solids concentration than is achieved using ordinary commercial formaldehyde, results in resins having a higher degree of water solubility, since there is then a tendency for more of the solubilizing groups to become part of the resin molecule. Such resins, when diluted after preparation, also have greater stability. A resin embodying the invention when reacted at a higher solids concentration than is achieved using ordinary commercial formaldehyde has a greater degree of water solubility (and stability, after dilution) than a resin reacted at a similar increased solids concentration but containing no glycol.

The solids concentration of the reaction mixture may be increased by using the neutralized substituted carboxylic acid in the form of its crystalline salt. For example, a resin embodying the invention prepared with crystalline sodium glycolate is more soluble and has better stability than a similar resin prepared with an equivalent amount of a solution of 70 per cent glycolic acid neutralized with flake caustic. Even greater improvement in the water solubility of resins embodying the invention is obtained if the concentration of solids in the reaction mixture is increased by using a formaldehyde solution containing a greater concentration of formaldehyde than 37 per cent. It is desirable to use an aqueous solution containing a concentration of 45 to 50 per cent of formaldehyde, since use of such a concentrated formaldehyde solution gives substantially improved properties economically and efficiently. If desired, paraformaldehyde may be dissolved in a 37 per cent aqueous formaldehyde solution to raise the concentration of formaldehyde to 45 or 50 per cent.

A commercial formaldehyde solution is in itself highly acid so that the pH of the reaction mixture containing also the hydroxy-substituted carboxylic acid is quite low. Since the reaction of formaldehyde and urea tends to go too rapidly in a strongly acid solution so that the product gels, and since the reaction does not proceed

satisfactorily if the solution is strongly alkaline, it is desirable that the pH of the reaction mixture be adjusted within the range 5.2 to 5.6. Varying the reaction pH between 5.2 and 5.6 and varying the reaction temperature has no substantial effect in general on the properties of resins reacted to the same degree of condensation. Since, however, undesirable by-products form within this pH range at temperatures below around 95 degrees C. it is desirable to lower the pH to within the range from 5.2 to 5.6 only after the temperature of the reaction mixture reaches about 95 degrees C., to avoid turbidity in the final product. (Although formation of an insoluble by-product has no effect on the wet-strengthened paper made from filtered resin, the presence of a precipitate makes colorimetric pH control during the resin preparation very difficult.) It is, therefore, most desirable to raise the initial pH with a base within a range of about 6.5 to 7.0 and to maintain the pH of the mixture in approximately this range until the temperature is about 95 degrees C.

It is preferable to use a strong base such as an alkali metal base (as hereinbefore defined). Such a base will also neutralize part or all of the hydroxy-substituted carboxylic acid. At the time of reaction it is preferred that from 20 to 100 mol per cent of the hydroxy-substituted carboxylic acid taking part in the reaction be in the form of a metal salt that is water soluble and does not interfere in the reaction. The product of such a reaction is a composition embodying the invention because the salt is largely ionized in the aqueous reaction medium, and some of the anions produced by such ionization combine with hydrogen ions to form molecules of the carboxylic acid so that some of the molecules taking part in the reaction are molecules of the free carboxylic acid. If the water present during the reaction is removed by drying the reaction product, and if the cations from the metal base are present in an amount sufficient to combine with all of the carboxy groups in the molecules of the reaction product, the ionization which took place when the alkali metal salt dissolved in the aqueous reaction medium is reversed during the drying of the reaction product and all the carboxy groups in the dried reaction product are neutralized by the metal base.

In the practice of the invention the resin components may be mixed in any desired order. It is usually desirable to neutralize the carboxylic acid first. The formaldehyde solution and the glycol may then be added and the mixture heated for about two hours, prior to the addition of urea and sufficient base to raise the pH within the range from 6.5 to 7.0. Alternatively the urea and formaldehyde solution may be adjusted to the proper pH and reacted for about 45 minutes prior to the addition of the neutralized hydroxy-substituted carboxylic acid and the glycol. The glycol may be added at some period during the reaction. It is preferable, however, to add it before starting the reaction. Most desirably the formaldehyde solution, urea and glycol are added successively to the neutralized hydroxy-substituted carboxylic acid, and additional base is then added to raise the pH of the mixture within the range from 6.5 to 7.0. The mixture then either may be heated for one hour at 60 degrees C. or may be allowed to stand overnight.

It is believed that during this preliminary reaction stage one molecule of formaldehyde combines with one molecule of water to form methyl-

ene glycol, and it is believed to be the methylene glycol that actually takes part in the reaction with a substance such as urea, so that a methylol group is formed by the condensation of a methylene glycol molecule with an NH<sub>2</sub> group in the urea molecule; one molecule of water being eliminated in such condensation:



Thermosetting compositions of the invention having equally as good properties may be obtained without this much preliminary reaction. It is necessary merely to allow enough time for the reactants to dissolve before continuing the reaction as hereinafter described.

In general, more highly condensed resins impart better wet strength to paper. However, the increase in wet strength imparted by a given resin may be inappreciable beyond a certain degree of condensation (viscosity), and since increased condensation tends to decrease both the stability and the water solubility of resins embodying the invention, the reaction should be terminated when that viscosity has been reached. The viscosity of resins reacted to the same degree of condensation will, of course, differ in accordance with the solids concentration of the reaction mixtures. Resins embodying the invention in which the proportions of resin reactants are the desirable proportions hereinbefore given and in which the concentration of formaldehyde in aqueous solution is approximately (a) 37 per cent, (b) 50 per cent or (c) 45 per cent are reacted to a desirable degree of condensation as follows:

(a) The pH of the reaction mixture is initially adjusted to 6.5-7.0, the mixture is heated to a temperature of about 95 degrees C. before lowering the pH to 5.2-5.6, and the reaction is continued at this temperature until the viscosity of the resin solution is about 27 seconds (measured by Ford Cup,  $\frac{3}{2}$  inch opening, at 25 degrees C.). The reaction usually requires about eight to nine hours when the pH is about 5.6, or from two to six hours when the pH is within the range 5.3 to 5.45. The mixture is then cooled to 60 degrees C. and held at this temperature until the viscosity of the solution is 32 to 34 seconds (Ford Cup), the pH being adjusted to 5.6 at the beginning of this period. This latter reaction stage usually requires from one to three hours.

(b) The pH of the reaction mixture is initially adjusted to 6.5-7.0, and the mixture is heated to a temperature of 95 degrees C., two subsequent pH adjustments being made, one to 7.5 at 50 degrees C. and the other to 7.2 at 75 degrees C. to avoid precipitate formation. It is desirable that the temperature rise from 65 degrees C. to 95 degrees C. in less than 45 minutes. The mixture is held at 95 degrees C. for five minutes before lowering the pH to about 5.6, and the solution is held at this temperature and pH until the viscosity of the resin solution is "J" (measured by Gardner - Holdt bubble viscometer - standard method, the Ford Cup viscosity method becoming increasingly inaccurate at the much higher viscosity encountered using the more concentrated reaction mixture). The mixture is then rapidly cooled to 60 degrees C. (about 10 minutes' cooling time) and held at this temperature until the viscosity of the solution is "V" - "W" (Gardner Holdt).

(c) The resin is prepared by the procedure de-

scribed in (b) except that the viscosity of the solution after the 95 degree stage should be "H"- "I," and the final viscosity after the 60 degree stage should be "U"- "V" (Gardner-Holdt).

Using a two-stage reaction (that is, heating first at 95 degrees C. to a certain viscosity and then reaching the final viscosity by reacting at 60 degrees C.) ordinarily makes the reaction more controllable and gives more reproducible results than a one-stage reaction carried to the same final viscosity at 95 degrees C., although there is no essential difference in the properties of the final product. Usually, the total reaction time must be at least three to four hours in order to allow sufficient time for the viscosity measurements and the temperature and pH adjustments that are necessary for safe control.

The wet strengthening properties of a resin of the invention may be appreciably increased by aging the resin for a period of time at room temperature or even lower temperatures. There is also a gradual improvement in solubility on aging. The type of condensation that takes place on aging at room temperature seems to differ from that which takes place during the actual reaction carried out at higher temperatures. During the reaction the cloud temperature (i. e., the temperature above which a drop of resin solution dissolves in a given amount of water leaving a substantially clear solution) gradually increases to a certain point where it tends to level off. On aging, resin samples show a gradual decrease in cloud temperature up to the point of gelling, at which there is a sharp increase in cloud temperature.

It is desirable to neutralize the liquid resin with a base such as sodium hydroxide to a pH of at least 7.0. Preferably the pH is adjusted to the range 7.8 to 8.0, for maximum stability. The pH of the resin solution decreases on standing, the decrease being more rapid at higher temperatures. The decreasing pH of the resin solution is probably at least partially due to the formation of formic acid through air oxidation (and Cannizzaro type reaction) of the free formaldehyde usually present. Therefore, a buffer such as sodium bicarbonate, sodium borate, or borax is usually added to retard the rate of pH drop. Although use of 0.5 per cent of borax (based on the weight of solids in the resin), or 0.5 per cent of sodium bicarbonate, or 0.2 to 0.3 per cent of sodium borate gives good results, it is more effective to add a buffer mixture containing 70 per cent boric acid and 30 per cent borax (in a ready prepared 10 per cent water solution) to the extent of 1 to 3 per cent (based on the weight of resin solids). Resins embodying the invention which are prepared using a more concentrated reaction mixture are most desirably adjusted to a pH of 8.0 and buffered with 2 per cent (based on the weight of solids in the resin) of a buffer mixture containing 65 per cent boric acid and 35 per cent borax.

Resins reacted according to the procedure described in (a) ordinarily contain about 48 to 50 per cent solids, and those reacted according to procedures (b) and (c) ordinarily contain about 51 to 55 per cent solids. The good stability of a resin embodying the invention can be further improved by diluting the resin so that the solids concentration is about 45 per cent. Although further dilution may improve the stability even more, this concentration seems most advantageous for shipping and storing the resin.

The magnitude of the improvement in wet strength imparted either by a thermosetting resin embodying the present invention or by a resin which is similar in every respect except that no glycol is used, over that imparted by the resins previously used for imparting wet strength, may be demonstrated by tests carried out as follows. The results of these tests are shown in Table 1.

Anhydrous sodium bisulfite (167 grams) is dissolved in methanol-free formalin (1960 grams of a solution consisting of 37 per cent formaldehyde and 63 per cent water). Urea (660 grams) and sodium acetate (4.5 grams) are dissolved in this solution in a 3 liter three-necked flask fitted as described above. The solution is allowed to stand overnight at room temperature. The solution is then heated on a boiling water bath for about eight and one-half hours at a temperature ranging from 94.5 degrees C. to 97.5 degrees C. (The buffer action of the sodium acetate keeps the pH at approximately 5.6 during the latter part of this heating period.) The mixture is allowed to stand overnight and is then held at a temperature of 60 degrees C. and at a pH of 5.6 for five hours before cooling to room temperature. This resin is resin A in Table 1, a resin of the type heretofore used for imparting wet strength (the control resin).

A hydroxy-substituted carboxylic acid (87.5 grams of glycolic acid in 37.5 cc. of water) is mixed with flake caustic (50 grams) and to this mixture in a 1 liter three-necked flask fitted with a thermometer, reflux condenser, stirring rod and oil seals is added urea (240 grams), a glycol (48 grams of glycerine) and methanol-free formalin (687 grams of an aqueous solution consisting of 37 per cent formaldehyde and 63 per cent water). The mixture is held at temperatures ranging from 94 to 98 degrees C. at a pH of 5.4 for three hours. The solution is then cooled to 60 degrees C. and held at this temperature for one hour before cooling to room temperature and neutralizing to a pH of 7.0 with sodium hydroxide. This resin is resin B in Table 1.

Resin C in Table 1 is prepared by the procedure used for resin B except that no glycerine is used.

Resins A, B and C are used to treat paper prepared and tested by the following procedure:

Pulp (containing the equivalent of 360 grams of oven-dried pulp) is soaked in water (10 liters) overnight. The soaked pulp is then agitated for 10 minutes with a "Lightnin" mixer (a high-speed motor-driven stirrer). The agitated suspension is then placed in a "Valley" beater (a standard beater designed for laboratory use) and enough water is added to bring the total volume of water to 23 liters (measured at a temperature of 25 degrees C.). The beater is run for five minutes (slush period) before a load (4500 grams) is placed on the lever arm which applies a force to the beater roll. Samples are withdrawn at various intervals during the beating to measure the rate at which water passes through the pulp (freeness) as Schopper freeness. The freeness of an 800 ml. sample after twenty minutes' beating time is about 700 and that for an 800 ml. sample after about thirty minutes' beating time is 550. The beating is terminated after thirty minutes.

The beaten pulp is diluted to such an extent that a volume of approximately 800 ml. gives a dry sheet weighing 2.0 grams. The pH is adjusted to 6.5 by the addition of sulfuric acid. Alum (a fresh solution of 17.76 grams of anhydrous aluminum sulfate in about 90 cc. of water) is added

with stirring to the beaten pulp suspension which is then ready for the addition of the resin for imparting wet strength. The beaten pulp suspension is allowed to stand for five minutes before a resin for imparting wet strength (an amount of a resin solution sufficient to give 3 per cent based on the weight of the dry pulp) is added. A volume of stock large enough to give a sheet of the desired 2.0 grams weight (800 ml.) is placed in the sheet machine and diluted to a total volume of 10.7 liters, and the pH is adjusted to 4.5 by addition of sulfuric acid. The handsheet is made within five minutes after the addition of the resin and the operation is repeated four times without delay, to make four more sheets.

The handsheets are made according to "Institute of Paper Chemistry-Tentative Method 411-B-Valley." The sheets are pressed separately between six blotters under a pressure of 100 pounds for two minutes. Each sheet is placed on the drier while still in contact with one blotter (sheet against the metal) and dried for five minutes at 250 degrees F. The sheets are conditioned for a minimum of eight hours in a room at a temperature of 75 degrees F., and at 78 per cent relative humidity before testing.

Wet strength measurements are made on the handsheets with a Mullen tester which measures the bursting pressure, expressed as points (approximately pounds per square inch) for a standardized circular area. Bursting strength of the paper is given herein as a burst factor, that is, points per 100 pounds of basis weight ("basis weight" is the weight of 500 sheets of the paper, 25 inches by 40 inches). Mullen wet burst values are obtained on paper samples wet with water from a brush (equivalent to about a ten-second soak of the paper samples).

TABLE 1

|              | Mullen<br>Wet Burst |
|--------------|---------------------|
| Resin A..... | 25.0                |
| Resin B..... | 33.7                |
| Resin C..... | 33.9                |

It may be readily seen from Table 1 that both resins B and C impart wet strength higher than that imparted by resin A and that there is essentially no difference in the wet strength imparted by resins B and C.

The magnitude of the improvement in the stability of a thermosetting composition embodying the invention (resin B) over that of a control resin containing no glycol (resin C) may be demonstrated by tests carried out as follows:

Samples of resins B and C are adjusted to a pH of 8.5 and held in an oven at a temperature of 78 degrees F. Other samples of resins B and C adjusted to the same pH are held at a temperature of 120 degrees F. Stability of these samples is indicated by the number of days the samples remain at these temperatures without gelling; the results being recorded in Table 2.

TABLE 2

|              | 78 degrees<br>F., days | 120 degrees<br>F., days |
|--------------|------------------------|-------------------------|
| Resin B..... | 210                    | 10                      |
| Resin C..... | 89                     | 4½                      |

The stability of a resin containing a glycol (resin B) is more than twice as great at either temperature than the stability of a resin (resin C) prepared in the same manner as resin B except that no glycol is used.

As hereinbefore demonstrated, not only are resins embodying the present invention capable of imparting greater wet strength to paper than the synthetic resins heretofore used for the impregnation of paper, but they also possess improved stability over resins which may impart equally as high wet strength. That resins embodying the invention have improved water solubility in addition to improved stability may be demonstrated by tests carried out as follows: (The results of these tests are shown in Table 3.)

A hydroxy-substituted carboxylic acid (252 grams of glycolic acid in 108 cc. of water) is mixed with flake caustic (132 grams), and the mixture is maintained for one-half hour at temperatures ranging from 70 to 80 degrees C. To the resulting sodium glycolate in a 3-liter three-necked flask fitted with a thermometer, reflux condenser, stirring rod, and oil seals is added methanol-free formalin (1981 grams of a solution consisting of 37 per cent formaldehyde and 63 per cent water), urea (690 grams) and a glycol (138 grams of glycerine). Flake caustic is added to adjust the pH into a range from 6.5 to 7.0.

The mixture is heated to a temperature of 90 degrees C. and the pH is lowered to approximately 5.3 by the addition of glycolic acid. The heating is continued at temperatures ranging from 95 to 96 degrees C. until the viscosity of the solution (Chrome Ford Cup, measured at 25 degrees C. using a  $\frac{3}{2}$  opening) is about 25.5 seconds (attained after about  $2\frac{1}{4}$  hours of heating). The mixture is cooled to a temperature of 60 degrees C. and the pH is raised to 5.6 by the addition of sodium hydroxide. The mixture is then held at this temperature until the viscosity measures about 31.5 seconds (after about 3 hours at 60 degrees C.). The resin is cooled to room temperature and neutralized with sodium hydroxide to a pH of 6.98 (glass electrode). This resin is resin K in Table 3.

The control resin, resin D, in Table 3, is prepared like resin K except that no glycerine is added. The mixture is reacted to a viscosity of 25.5 seconds by heating for one hour and 40 minutes at temperatures ranging from 95 to 97 degrees C., and a viscosity of 31 seconds is reached after the mixture has been cooled to 60 degrees C. (the pH being adjusted to 5.6) and held at this temperature for one hour. The resin is cooled to room temperature and neutralized with sodium hydroxide to a pH of 7.05 (glass electrode).

The per cent solids in the resins (determined by curing a weighed sample of the liquid resin on a glass plate and weighing the dried sample) is 48.6 in resin K and 48.5 in resin D. The viscosity is 32 seconds for resin K and 32.5 seconds for resin D.

Test tube portions of resin K and resin D are diluted with distilled water to various concentrations of solids. Solubility is determined by cooling the sample in an ice bath until a two-phase system forms, warming the test tube and noting the temperature at which the solution forms a one phase system. Solubility data are recorded in Table 3 in terms of the "cloud temperature," i. e., the temperature above which the one-phase water solution is formed at the given solids concentration.

13  
TABLE 3

| Percent Solids | Cloud Temperature, ° C. |         |                      |         |
|----------------|-------------------------|---------|----------------------|---------|
|                | Resin K                 | Resin D | 1 mo. aging—buffered |         |
|                |                         |         | Resin K              | Resin D |
| 30             | 10                      | 19.5    |                      |         |
| 25             | 13                      | 22.5    | 8.5                  | 18      |
| 23             | 14.5                    | 23.5    | 10                   | 19      |
| 20             | 15                      | 24.5    | 11.5                 | 20      |
| 15             | 16                      | 24.5    | 12                   | 20.5    |
| 10             | 13.5                    | 21      | 9.5                  | 16.5    |

A comparison of the solubility of resins K and D after preparation is shown in column 2 and 3 in Table 3.

Columns 4 and 5 show the cloud temperatures of samples of these resins after aging 1 month at "cold room" temperature. These samples are prepared by first adjusting the pH with sodium hydroxide to 8.0 (Beckman pH meter) and then adding 2 per cent (based on weight of resin solids) of a buffer mixture consisting of 40 per cent sodium borate and 60 per cent borax.

From the table it may be seen that resin K (containing a glycol) is more soluble in water than the control (resin D) at every solids concentration, and that the cloud temperature of resin D is approximately one and one-half times as high as that for resin K at every solids concentration. The cloud temperature of all samples decrease about 3 or 4 degrees during one month of aging.

The improvement in stability of a resin embodying the invention (resin K) over a resin containing no glycol (resin D) is demonstrated by the results of tests made on samples of these resins adjusted with sodium hydroxide to various pH values (determined with a Beckman pH meter) and buffered with a sodium borate-boric acid mixture. Each sample is divided into three portions which are placed at temperatures of 78 degrees F., 90 degrees F. and 120 degrees F., respectively, to obtain the stability results shown in Table 4. Table 5 shows the results of stability tests on samples of the liquid resins diluted with distilled water to various solids concentrations.

TABLE 4

| Resin samples | Days (1% buffer) |        |         | Days (2% buffer) |        |         |
|---------------|------------------|--------|---------|------------------|--------|---------|
|               | 78° F.           | 90° F. | 120° F. | 78° F.           | 90° F. | 120° F. |
| K-1           | 71               | 48     | 12½     | 54               | 36     | 10½     |
| D-1           | 57               | 37     | 9½      | 50               | 33     | 8½      |
| K-2           | 96               | 62     | 16½     | 71               | 46     | 15      |
| D-2           | 37               | 23     | 7½      | 46               | 29     | 8       |
| K-3           | 85               | 55     | 23½     | 82               | 53     | 16      |
| D-3           | 20½              | 12½    | 5½      | 32               | 23     | 7       |

Columns 2, 3 and 4 show tests made on 200 gram samples containing 1 per cent buffer, based on weight of resin solids, as follows: Sample 1: each resin adjusted to pH 8.0 before addition of a buffer mixture consisting of 40 per cent sodium borate and 60 per cent boric acid; sample 2: pH of 8.5, 70 per cent sodium borate, 30 per cent boric acid; sample 3: pH 9.0, 100 per cent sodium borate. Columns 5, 6 and 7 show tests made 16 days later on 150 gram samples containing 2 per cent buffer (based on weight of resin solids) as follows: Sample 1: each resin adjusted to pH 7.75 before addition of a buffer mixture consisting of 30 per cent sodium borate and 70 per cent boric acid; sample 2: pH 8.0, 40 per cent sodium

borate, 60 per cent boric acid; sample 3: pH 8.25, 53 per cent sodium borate, 47 per cent boric acid.

The results in Table 4 indicate that the stability at 90 degrees F. is 3 to 4 times the stability at 120 degrees F., and that the stability at 78 degrees F. is about 5 to 6 times the stability at 120 degrees F. Resin K has better stability than resin D at every temperature and with every pH adjustment and buffering combination tested.

TABLE 5

| Resin | Percent Solids | Days Stable |        |         |
|-------|----------------|-------------|--------|---------|
|       |                | 78° F.      | 90° F. | 120° F. |
| K     | 49             | 27          | 15     | 4½      |
| K     | 45             | 30          | 19     | 6½      |
| K     | 40             | 33          | 22     | 7½      |
| D     | 49             | 26          | 14     | 3       |
| D     | 45             | 27          | 17     | 5½      |
| D     | 40             | 28          | 19     | 6½      |

The stability of both resins K and D increase upon dilution from 49 per cent solids concentration to 40 per cent solids concentration, the stability of resin K being greater than that of resin D at each concentration and temperature tested.

The following examples illustrate the practice of the invention:

*Example 1*

A resin embodying the invention is prepared by one of the following procedures in which the glycol is not initially reacted with the other resin components.

(a) A hydroxy-substituted carboxylic acid (70 grams of glycolic acid in 30 cc. of water), flake caustic (33 grams), methanol-free formalin (713 grams of a solution consisting of 37 per cent formaldehyde and 63 per cent water) and urea (240 grams) are mixed in a 1-liter three-necked flask equipped with a thermometer, reflux condenser, stirring rod and oil seals. The mixture is held at a temperature of about 96 degrees C. for two and one-half hours, the pH of the mixture being adjusted to 5.4 with glycolic acid as soon as the temperature is above 90 degrees C. A glycol (48 grams of glycerine) is then added, and the mixture is cooled to 60 degrees C., and held at this temperature for one hour. The pH is raised to 5.6 at the beginning of this period by the addition of flake caustic. The resin is cooled to room temperature, neutralized to a pH of 7.5 with flake caustic, and buffered by addition of sodium bicarbonate (6 grams).

(b) A hydroxy-substituted carboxylic acid (87.5 grams of glycolic acid in 37.5 cc. of water), flake caustic (50 grams), methanol-free formalin (687 grams of a solution consisting of 37 per cent formaldehyde and 63 per cent water) and urea (240 grams) are mixed and heated for three hours at a temperature of 95 degrees C (pH 5.4) by the procedure described in (a). The mixture is then cooled to 60 degrees C. and held at this temperature for one-half hour before cooling to room temperature, neutralizing to a pH of 7.0 and buffering by addition of triethanolamine (2.6 grams). A glycol (48 grams of ethylene glycol) is then added.

(c) Other resins for imparting wet strength having good stability and water-solubility, are prepared by a procedure that is the same as the procedure described in (b) except that the ethylene glycol is replaced with an equivalent amount of one of the following glycols: diethylene glycol, propylene glycol, or pentaerythritol.

## Example 2

A resin embodying the invention is prepared by one of the following procedures in which the glycol is initially reacted with the other resin components.

(a) A hydroxy-substituted carboxylic acid (87.5 grams of glycolic acid in 37.5 cc. of water), flake caustic (50 grams), methanol-free formalin (687 grams of a solution consisting of 37 per cent formaldehyde and 63 per cent water), a glycol (58 grams of diethylene glycol) and urea (240 grams) are mixed in a 1 liter three-necked flask fitted with a thermometer, reflux condenser, stirring rod and oil seals. The mixture is reacted for three and one-half hours at a temperature of 95 degrees C., the pH being adjusted with additional glycolic acid to about 5.4 immediately after the temperature reaches 90 degrees C. The solution is then cooled to 60 degrees C. and held for one and one-half hours at this temperature. After cooling the resin to room temperature, it is neutralized with sodium hydroxide to a pH of 7.0 and buffered by addition of triethanolamine (2.6 grams).

This procedure for producing a water soluble, stable resin for imparting wet strength may be carried out using tartaric acid (150 grams) or lactic acid (90 grams) in place of the glycolic acid.

(b) A resin having even greater water solubility and stability than the one whose preparation is described in (a) may be prepared by substituting ethylene glycol (58 grams) in place of the diethylene glycol. The mixture is reacted for four hours at 95 degrees C., the pH being adjusted to 5.3 with glycolic acid as soon as the temperature is above 90 degrees C. The solution is then cooled to 60 degrees C. and held for three-quarters of an hour at this temperature before cooling to room temperature. The resin is neutralized with sodium hydroxide to a pH of 7.0 and buffered by addition of triethanolamine (2.6 grams).

(c) A hydroxy-substituted carboxylic acid (252 grams of glycolic acid in 108 cc. of water) is mixed with flake caustic (100.3 grams in 31.7 cc. of water) and the mixture is held at temperatures ranging from 75 to 80 degrees C. (for fifteen minutes). To the resulting sodium glycolate solution in a flask as described in (a) is added a glycol (138 grams of glycerine), methanol-free formalin (1980 grams of a solution consisting of 37 per cent formaldehyde and 63 per cent water) and urea (690 grams). The pH of the mixture is adjusted to approximately 7.4 (Beckman pH meter) by the addition of flake caustic. The mixture is then heated to 90 degrees C. and glycolic acid is added to lower the pH to about 5.6. The solution is reacted to a viscosity of 32.5 seconds (measured with a Chrome Ford Cup,  $\frac{3}{8}$  inch opening, at 25 degrees C.) by holding at temperatures ranging from 92 to 95 degrees C. for about two and three-quarters hours, the pH being about 5.5 during the first half of this period and about 5.4 during the last half. The solution is then cooled to 60 degrees C., the pH is raised to 5.6 by the addition of sodium hydroxide, and the solution is held at a temperature of about 61 degrees C. until the viscosity is slightly greater than 33 seconds (about 1 hour at this temperature). The resin is then cooled to room temperature, the pH is adjusted to 7.8 with flake caustic, and sodium bicarbonate (16  $\frac{1}{2}$  grams) is added.

(d) A hydroxy-substituted carboxylic acid (87.5 grams of glycolic acid in 37.5 cc. of water) is neutralized with sodium hydroxide (50 grams)

by the procedure described in (c). To the resulting sodium glycolate solution is added a glycol (50 grams of pentaerythritol), methanol-free formalin (697 grams of a solution consisting of 37 per cent formaldehyde and 63 per cent water) and urea (240 grams). The pH is adjusted to 6.8 with additional sodium hydroxide and the mixture is heated to a temperature of 90 degrees C. The pH is then adjusted to 5.4 with glycolic acid and the mixture is held for two and one-half hours at about 95 degrees C. The mixture is then cooled to 60 degrees C. and held at this temperature for one-half hour, the pH being raised to 5.6 with sodium hydroxide during the last fifteen minutes. The resin is cooled to room temperature, neutralized with sodium hydroxide to pH 7.1, and buffered by addition of sodium bicarbonate (5 grams).

## Example 3

The following procedures further illustrate the practice of the invention:

(a) A hydroxy-substituted carboxylic acid (90 grams of lactic acid in 90 cc. of water) is neutralized by mixing with sodium hydroxide (50 grams) for fifteen minutes at a temperature maintained between 75 and 80 degrees C. To the resulting sodium lactate solution is added methanol-free formalin (687 grams of a solution consisting of 37 per cent formaldehyde and 63 per cent water) and the mixture is held at 95 degrees C. for two hours, in a 1 liter three-necked flask equipped with a thermometer, reflux condenser, stirring rod and oil seals, the pH being adjusted to 6.0 at the beginning of the period. A glycol (50 grams of glycerine) and urea (240 grams) are then added, the pH is adjusted to 5.4 with lactic acid and the solution is held for five and one-half hours at a temperature of about 95 degrees C. The resin is then cooled to room temperature and neutralized with sodium hydroxide to a pH of about 7.8.

(b) A hydroxy-substituted carboxylic acid (87.5 grams of glycolic acid in 37.5 cc. of water), flake caustic (50 grams), a glycol (48 grams of glycerine) and methanol-free formalin (252 grams of a solution consisting of 37 per cent formaldehyde and 63 per cent water) are mixed in a 1 liter three-necked flask equipped with a thermometer, reflux condenser, stirring rod and oil seals, and the mixture is held for two hours at 95 degrees C., the pH being adjusted to 5.5 at the beginning of this period. Urea (240 grams) is then added, the pH is adjusted to 6.5 with sodium bicarbonate and the mixture is allowed to stand for fifteen minutes before adding methanol-free formalin (435 grams of a solution consisting of 37 per cent formaldehyde and 63 per cent water). The heating is then continued for four and three-quarters hours at about 95 degrees C., the pH being lowered to 5.4 at the beginning of this heating period by the addition of glycolic acid. The resin solution is then cooled to room temperature and neutralized with sodium hydroxide to a pH of 7.8.

(c) A hydroxy-substituted carboxylic acid (70 grams of glycolic acid in 30 cc. of water), flake caustic (33 grams), methanol-free formalin (687 grams of a solution consisting of 37 per cent formaldehyde and 63 per cent water), a glycol (24 grams of glycerine) and urea (240 grams) are mixed and reacted as described in Example 2(a) except that the mixture is held at 96 degrees C. for two hours and the heating period at 60 degrees C. is two hours at a pH of 5.6 (raised with

sodium hydroxide). The resin is neutralized with sodium hydroxide to a pH of 7.5 and buffered by addition of sodium bicarbonate (6 grams).

(d) A hydroxy-substituted carboxylic acid (70 grams of glycolic acid in 30 cc. of water), flake caustic (33 grams), methanol-free formalin (713 grams of a solution consisting of 37 per cent formaldehyde and 63 per cent water), a glycol (48 grams of glycerine) and urea (240 grams) are mixed and heated as described in (c) for two and one-half hours at 96 degrees C. and one and one-half hours at 60 degrees C. The resin is neutralized with sodium hydroxide to a pH of 7.5 and buffered by addition of sodium bicarbonate (6 grams).

(e) Urea (720 grams) and methanol-free formalin (2064 grams of a solution consisting of 37 per cent formaldehyde and 63 per cent water) are mixed in a 3 liter three-necked flask fitted with a thermometer, reflux condenser, stirring rod and oil seals. A glycol (144 grams of glycerine) is added, and the pH of the mixture is adjusted with sodium hydroxide within the range 6.5 to 7.0. Crystalline sodium glycolate (174 grams of the monohydrate) is added and the mixture is then heated to a temperature of 97 degrees C. before lowering the pH to 5.3 by the addition of glycolic acid. The heating is continued at temperatures ranging from 93 to 95 degrees C. until the viscosity of the solution is 36.5 seconds (measured by Ford Cup method, attained after about two and three-quarters hours of heating). The solution is cooled to 60 degrees C., the pH is raised to 5.6 with sodium hydroxide, and the solution is maintained at this temperature and pH until the viscosity is 52 seconds (attained after approximately two hours at 60 degrees C.). The resin is cooled to room temperature, the pH is adjusted to 8.5 with sodium hydroxide, and a buffer (0.686 gram of sodium borate mixed with 0.294 gram of boric acid) is added.

(f) A hydroxy-substituted carboxylic acid (375 grams of a solution consisting of 70 per cent glycolic acid and 30 per cent water) is neutralized with flake caustic (138 grams) by mixing for fifteen minutes at temperatures maintained at about 75 to 80 degrees C. To the resulting sodium glycolate solution in a 3 liter three-necked flask fitted with a thermometer, reflux condenser, stirring rod and oil seals is added methanol-free formalin (1526 grams of a solution consisting of 50 per cent formaldehyde and 50 per cent

water, prepared by vacuum distillation of commercial 37 per cent formalin), urea (720 grams) and glycerine (144 grams). The mixture is heated to a temperature of 90 degrees C. before the pH is lowered to 5.5 with glycolic acid. The heating is continued at approximately 95 degrees C. for one hour. The solution is then cooled to 60 degrees C. and held at this temperature for about one hour. The resin is cooled to room temperature and diluted to about 45 per cent solids (with approximately 400 ml. of distilled water), and the pH is adjusted to 7.8 with sodium hydroxide. A buffer (0.164 gram of borax mixed with 0.381 gram of boric acid) is added to the resin solution.

I claim:

1. A paper treating resin of improved stability and solubility in dilute aqueous solution that is capable of imparting superior wet strength to paper, comprising a water-soluble intermediate condensation product of (a) formaldehyde, (b) urea, said formaldehyde and urea being in a proportion of one mol of urea for each 1.9-2.15 mols of formaldehyde, (c) an alkali metal salt of glycolic acid, said alkali metal salt of glycolic acid being in a proportion of 0.15-0.25 mol for each mol of urea, and (d) a polyhydric alcohol of the class consisting of polyhydroxy alkanes and linear ethers thereof whose molecule has from 2-10 atoms, has not more than two carbon atoms per hydroxy group and has no constituents other than hydroxy groups, said polyhydric alcohol being 10-20% by weight of the amount of said urea.

2. A paper treating resin as claimed in claim 1 wherein said polyhydric alcohol is glycerol.

#### References Cited in the file of this patent

#### UNITED STATES PATENTS

| Number    | Name     | Date          |
|-----------|----------|---------------|
| 2,317,181 | D'Alelio | Apr. 20, 1943 |
| 2,322,887 | Schwartz | June 29, 1943 |
| 2,322,888 | Schwartz | June 29, 1943 |
| 2,374,812 | Gutkin   | May 1, 1945   |
| 2,389,415 | D'Alelio | Nov. 20, 1945 |
| 2,524,111 | La Piana | Oct. 3, 1950  |

#### FOREIGN PATENTS

| Number  | Country       | Date          |
|---------|---------------|---------------|
| 320,915 | Great Britain | Oct. 28, 1929 |
| 535,745 | Germany       | Oct. 19, 1931 |
| 933,891 | France        | Jan. 5, 1948  |